# EUROPEAN PATENT SPECIFICATION

(11) **EP 0 788 558 B1**
(45) Date of publication and mention of the grant of the patent: **10.02.1999**
(21) Application number: 95931106.9
(22) Date of filing: 19.09.1995
(51) Int. Cl.: C22C 1/02, B01F 3/12, B01F 7/16

(54) **METHOD AND APPARATUS FOR ADDING ALUMINUM AND CALCIUM TO MOLTEN LEAD**
VERFAHREN UND VORRICHTUNG ZUM EINBRINGEN VON ALUMINIUM UND KALZIUM IN FLÜSSIGESBLEI
PROCEDE ET APPAREIL PERMETTANT D'AJOUTER DE L'ALUMINIUM ET DU CALCIUM A DU PLOMB FONDU

(30) Priority: 20.09.1994 CA 2132485
(43) Date of publication of application: 13.08.1997
(73) Proprietor: TIMMINCO LIMITED, Toronto Ontario M5W 1G5 (CA)
(72) Inventor: HIBBINS, Stephen, George, Renfrew, Ontario K7V 3V8 (CA); TIMPANO, Fernando, Anthony, Pembroke, Ontario K8A 1T8 (CA); ZULIANI, Douglas, John, Stitsville, Ontario K2C 1E5 (CA)
(74) Representative: Jehan, Robert
(86) International application number: CA9500525
(87) International publication number: WO9609418

(56) References cited:
- CA-A- 1 303 361
- US-A- 1 386 503
- US-A- 3 741 754
- US-A- 4 439 398

## Description

### Technical Field

This invention relates to a method for simultaneous addition of aluminum and calcium and alloys thereof to molten lead for the production of lead-calcium alloys.

### Background Art

Lead acid batteries historically have been produced with lead-antimony alloy grids. These lead-antimony batteries generate hydrogen gas through a chemical reaction with water in the electrolyte. This necessitates venting the battery and periodic replenishment of the water.

The introduction of lead-calcium alloy grids was a major development since these alloys greatly reduce the amount of hydrogen gas generated by the electrochemical reaction. As little as 0.1% calcium in the lead alloy is sufficient to reduce gassing to a level where the battery can virtually be sealed and no water additions are required.

The addition of calcium metal to lead is rather straightforward and can be accomplished by several methods including the simple addition of pure calcium metal or calcium alloys to the surface of a lead bath. Stirring the lead promotes better dissolution and minimizes opportunities for calcium oxidation as it floats on the surface of the lead melt.

U.S. Patent No. 3,741,754, which issued June 26, 1973 to C.M. Mainland, describes a process for adding granulated calcium metal to lead under an inert protective gas covering thereby minimizing oxidation of calcium during the addition. This process has the advantage of enabling calcium to be added to lead with high recovery and minimal fuming, emissions, flaring and losses to oxidation.

Alternatively, calcium may be introduced by adding calcium carbide as in U.S. Patent No. 1,941,534 to Betterton, which issued January 2, 1934.

The metallurgical difficulty with producing lead-calcium alloys is not in general related to the addition of calcium to molten lead since, as discussed above, there are several alternative alloying methods. The major problems relate to the fade of calcium once it has been dissolved in the liquid lead pool. Lead-calcium alloys are very prone to the loss of calcium due to oxidation at the melt surface where reactive calcium dissolved in the molten lead comes in contact with oxygen in atmospheric air.

A solution to the problems associated with calcium fade is given by the addition of minor amounts of aluminum (0.005% to 0.05%) to the lead-calcium alloy. Aluminum forms a tenacious oxide layer on the surface of the lead alloy melt thereby minimizing the oxidation of calcium.

Unlike calcium, however, the addition of aluminum to molten lead is quite difficult, being hindered by two factors:
a) a tenacious thin oxide film on the surface of solid aluminum metal which retards its dissolution rate in lead, and
b) aluminum's extremely low solubility in molten lead. At typical lead processing temperatures (400-600°C), the maximum solubility of aluminum in molten lead is only marginally higher than specifications for calcium-aluminum-lead alloys (up to 0.05% Al).

To add pure solid aluminum metal to lead effectively, the molten lead temperature has to be raised above aluminum's melting point (660°C) which is considerably higher than the normal range for lead processing. Due to its reactive nature, calcium metal is usually added at about 420°C. Hence there is an incompatibility between the melt temperatures at which solid aluminum and calcium metals can be added. Alternatively, pre-melted liquid aluminum can be poured and stirred into the lead bath; however, this requires a second furnace to melt the aluminum.

All of these higher temperature addition methods suffer from excessive oxidation, flaring and fuming leading to health and environmental concerns due to the presence of lead oxide fumes in the atmosphere. Because of the high melt temperatures, calcium recoveries are generally low, averaging below 85%, with aluminum recoveries ranging between 45% to 65%.

Other more environmentally acceptable methods have been developed, the most common utilizing the simultaneous addition of calcium and aluminum in the form of a eutectic alloy. An example of such a process is described in U.S. Patent No. 4,439,398 to Prengaman issued March 27, 1984. A suitable low melting point (545°C) eutectic alloy forms at 73% Ca/27% Al.

The eutectic alloy allows for simultaneous addition of calcium and aluminum in a ratio of approximately 3 Ca:1 Al at molten lead temperatures of about 570°C. Typically, reagent recoveries with this alloy are higher than for the pure calcium and aluminum metal addition practices outlined above; calcium and aluminum recoveries of 90% and 70% respectively can be expected with the alloy. The major difficulty arising with the use of this alloy is, however, that the addition ratio is 3 Ca:1 Al which often does not correspond to the proportion of calcium and aluminum required by the lead alloy specifications. In many cases, the desired Ca:Al ratio in the final lead alloy can be as high as 10:1. Achieving this addition ratio is difficult with an alloy of Ca and Al since the melting points of these alloys increase sharply on either side of the 73% Ca, 27% Al eutectic. These elevated melting points make off-eutectic alloys difficult to produce and difficult to use since the lead bath temperature must be increased accordingly. The disadvantages of higher lead temperatures include higher energy costs, longer processing times, shorter kettle life, higher calcium fade and increased lead oxide fume emissions.

Other technologies have also been developed to add aluminum and calcium to molten lead. U.S. Patent No. 4,808,376, issued February 28, 1989 to Worcester et al., adds calcium and aluminum powders by injecting a mixture carried by a stream of inert gas through a hollow lance which is submerged in a bath of molten lead. Because of the large density difference between the calcium and aluminum powders and liquid lead, the lance has to be equipped with a perforated canister at its tip. This canister acts to capture and hold the rising calcium and aluminum powders as they exit the lance. With this technique, calcium and aluminum recoveries are typically 90% and 55% respectively. This process still suffers from low aluminum recoveries and requires complicated and costly submerged injection equipment including the use of lances which are prone to plugging problems.

U.S. Patent 4,627,961, issued December 9, 1986 to Dudek, calls for the simultaneous addition of calcium and aluminum by compressing a mechanical mixture of the respective metal granules into a briquette. The briquettes are then added into a vortex created by stirring molten lead at temperatures between 550 and 600°C. The major difficulty with this method is unpredictability in the amount of calcium and aluminum recovered in the melt. Trials with calcium/aluminum briquettes, described in column 1 of aforesaid U.S. Patent No. 4,808,376, show highly variable results with calcium recoveries varying by up to 10% and aluminum recoveries varying by over 34%.

U.S. Patent No. 4,699,764, issued October 13, 1987 to Tobias et al., describes a complicated system where lead is melted in a separate holding furnace which is connected to a dissolution furnace by heated feed and return pipes. A pump is used to move the molten lead through the heated feed pipe in which the lead temperature is increased to the desired alloying temperature. The heated lead then passes through the dissolution furnace where it alloys with the addition reagents such as aluminum. The alloyed lead is then returned via the second pipe to the main lead holding furnace. The molten lead is continually circulated until the desired alloy composition is attained. This process is not only complicated but uses pumps and heated pipes which are maintenance intensive items.

In summary, while the addition of calcium metal to lead is relatively straightforward with recoveries of 90% or better expected, the addition of aluminum metal to molten lead is quite difficult. All processes which add pure aluminum metal at melt temperatures of 660°C or less (that is below the melting point of aluminum) suffer from low and highly variable aluminum recoveries. Many require complicated, costly and maintenance intensive equipment. At lead melt temperatures above aluminum's melting point, aluminum recoveries improve but the excessive heat leads to higher energy costs, longer processing times, shorter kettle life, higher calcium fade and excessive fuming of lead oxide causing serious environmental concerns.

### Disclosure of Invention

The present invention utilizes a simple system for simultaneous addition of calcium and aluminum metals at normal lead processing temperatures (typically 560°C and in any event below 660°C) with high and predictable recoveries and minimal oxidation and fume emissions.

High and predictable aluminum recoveries at melt temperatures below 660°C are unexpected since all previously described technologies resulted in low and/or highly variable aluminum recovery. In this regard, U.S. Patent No. 4,808,376 which adds pure calcium and aluminum metals by simultaneous addition through a submerged lance achieved average aluminum recoveries of 55% ranging between 44% and 62.5%. The preferred range of lead melt temperatures with this technology is between 550°C to 580°C.

Trials utilizing pure calcium/aluminum metal briquettes, reported in aforesaid U.S. Patent No. 4,808,376, column 1, were highly unpredictable reporting aluminum recoveries of on average about 71% but with a variability of ± 17% giving a 34% swing in aluminum levels. Lead bath temperatures of at least 550°C are recommended.

Other methods tor adding pure aluminum required that the lead be heated to temperatures above 660°C or that molten aluminum be added to the lead bath. These high temperature methods result in high calcium fade and excessive lead oxide fuming.

The present invention makes use of the exothermic release of heat provided when calcium metal dissolves in molten lead. When adding calcium particles, the heat release associated with calcium dissolution will cause a sharp local increase in the temperature of the lead surrounding the dissolving calcium particles. Since high melt temperatures are required to dissolve aluminum in lead, any aluminum particles coming in contact with the locally superheated lead adjacent to a calcium particle will dissolve rapidly.

To facilitate this increased aluminum dissolution rate, it is necessary to ensure that the calcium and aluminum particles are always maintained in close proximity with each other so that the heat released from the dissolving calcium particles is readily available to superheat the lead directly adjacent to an aluminum particle.

None of the previously described prior art for adding aluminum and calcium to molten lead at melt temperatures below about 660°C is designed to ensure calcium and aluminum particles are held within close proximity to each other throughout the dissolution reaction.

In accordance with a first aspect of this invention, there is provided a process of making a lead-calcium alloy as specified in claim 1.

As indicated above, the temperature of the lead bath will normally be less than 660°C.

A further aspect of the invention is an apparatus for introducing calcium and aluminum into a bath of molten lead as specified in claim 5 or 8.

As indicated, proper swirling of the lead is partially dependent on the shape of the housing and partially dependent on the nature and position of the impeller. The housing is constricted to impede flow of lead through the bottom opening and to assist in recirculation. Preferably, the lower portion of the tubular housing converges downwardly, providing a conical constriction leading to an outlet opening which may be about one half the maximum diameter of the housing and may be less than the impeller diameter. This helps to promote radial liquid flow to ensure that the calcium and aluminum particles are held in the tubular housing for an adequate length of time.

The design and location of the impeller is critical to establishing optimum liquid flow patterns inside the tubular housing. In the preferred embodiment, the impeller is located inside the housing just above the bottom opening, or at least closer to the bottom outlet than to a mid point of the downwardly converging portion. With this design, net liquid flow is downwards with liquid lead drawn in from the bulk melt through the top openings, swirled around inside the housing and forced out through the bottom opening. In this embodiment, the conical constriction in the bottom portion of the tubular housing is extremely important since it restricts the flow of lead through the bottom opening and thereby promotes radial flow. Without this constriction in the diameter of the tubular housing, the vortex would favour more axial flow thereby enabling calcium and particularly aluminum solid particles to escape the housing before being completely dissolved into the lead.

In a second embodiment, the impeller is located near the point of constriction inside the tubular housing. With this design, flow inside the housing reverses with liquid lead from the bulk melt being drawn in through the bottom opening and passing out of the top openings. In this case, the canopy above the top openings ensures that any unreacted calcium and aluminum particles which may be inadvertently discharged through the top openings are caught in the canopy because of their high buoyancy relative to lead and are thereby prevented from floating to the surface of the lead bath where they would be lost as unreacted reagent.

Unlike in U.S. Patent No. 3,741,754 aforesaid, which uses a marine type impeller to produce axial flow, the rotary impeller used in both embodiments herein is preferably at least partially of the centrifugal type, so that the lead in the region of the impeller is caused to move both radially and axially and to strike the walls of the tubular housing, and to swirl around adjacent to the wall before leaving the outlet. Also, unlike in the aforesaid '754 patent, the tubular housing is constricted in diameter so as to decrease axial flow and promote more radial flow within the housing. This is an important aspect of the present invention since it increases residence time of the aluminum and calcium particles inside the tubular housing. These features ensure that the particles are held within the tubular housing and retained in contact with a relatively small volume of lead while the exothermic reaction between the calcium heats this volume of lead to a temperature at which the aluminum dissolves.

While the invention is principally concerned with addition of particles of aluminum and calcium metals to the lead, the same process and apparatus can be used to add particles of aluminum/calcium alloy to lead, or a mixture of alloy and metal.

### Brief Description of the Drawings

The present invention will further be described with reference to the accompanying drawings, in which:
Fig. 1 is a partial view of prior art apparatus shown in U.S. Patent No. 3,741,754 as aforesaid;
Fig. 2 is a sectional elevation of apparatus in accordance with a preferred embodiment of this invention.
Fig. 3 is a sectional elevation of apparatus in accordance with a second embodiment of this invention

### Modes for Carrying Out the Invention

Fig. 1 shows the essential elements of prior art U.S. Patent No. 3,741,754 used for adding reactive metal, such as calcium, to molten lead while using a protective gas covering provided by an inert gas. As shown, a supply chute 12 forming the lower end of a feed hopper is used to deliver a supply of the reactive material. A cylindrical housing 16 which is closed at its top end 17 and open at its bottom end 18 is supported by support arm 20 from a movable frame 24. An inner chamber 26 is centrally disposed within housing 16. Within chamber 26 is located an impeller 28 of the marine or axial flow type attached to rotary shaft 29, which shaft extends up through gland 30 and has its upper end driven by a motor/gear box combination also mounted on frame 24. A vibrator 31 is connected to the base of chute 12 to assist flow of the reactive metal into the lead bath 32. An inert gas stream is provided through supply conduit 33; this assists movement of reactive particles into the top of housing 16. Frame 24 is arranged to be movable over a molten metal bath to be treated.

In use, the frame 24 is positioned to insert part of housing 16 and all of inner chamber 26 below the surface 32 of the molten lead. Inert gas is supplied through conduit 33, and the lead temperature adjusted to 900 to 950°F (i.e. 482 to 510°C). Calcium particles are supplied at a rate of about 115 grams per second (about 15 pounds per minute), while the impeller 28 is rotated at about 280 rpm to produce a deep vortex in the bath. The impeller tends to pull liquid lead upwardly through the annular space between the housing 16 and the inner chamber 26 and then downwardly through the chamber and out through its bottom outlet into the bath. The calcium particles are mixed with the molten lead during this movement. Using this apparatus, calcium-lead alloys were reportedly made ranging in calcium content from about 0.025% to 1.5% by weight calcium, based on the combined weight of calcium and lead in the alloy. The prior patent also reported that the addition of 6 mesh calcium nodules at a rate of about 115 grams per second (about 15 pounds per minute) to a lead bath at 480-510°C produced calcium recovery of about 88% by weight, i.e. about 88% of all calcium input became a part of the calcium-lead alloy.

At a preliminary stage of this invention, experiments were conducted to determine if the method as described in U.S. Patent No. 3,741,754 could be adapted to also add aluminum metal to lead. A reaction vessel similar to that reported in the patent and as shown in Fig. 1 herein was constructed. The reagent feed system was altered to facilitate the addition of:
* calcium and aluminum metal particles simultaneously, or,
* only aluminum metal particles.

Tests with this method, but at a temperature of 560°C, showed that when aluminum metal was added separately, that is without calcium addition, the aluminum recovery was zero. Hence this method is unsuitable for adding only pure solid aluminum metal particles to molten lead at processing temperatures customarily used for producing lead acid battery alloys.

Tests were also conducted using this method for simultaneously adding calcium and aluminum particles to the lead bath; the results are shown in Table 1 below.

**Table 1:**

| **Calcium and Aluminum Metal Recoveries with Simultaneous Addition Using the Method Described in U.S. Patent No. 3,741,754** | | | |
|---|---|---|---|
| Lead Temp. °C | Number of Tests | % Recovery | |
| | | Calcium | Aluminum |
| 500 | 4 | 86.6 ± 17.4 | 39.0 ± 19.9 |
| 540 | 3 | 90.6 ± 6.0 | 48.8 ± 7.2 |
| 560 | 9 | 91.9 ± 6.8 | 60.0 ± 9.6 |

The results in Table 1 prove that when aluminum and calcium particles are moved within close proximity to each other inside a well stirred cylindrical reaction bell or housing, the heat released by calcium dissolution locally increases the lead temperature in the vicinity of the aluminum particles thereby facilitating aluminum dissolution which would not have normally taken place in the absence of calcium.

The data in Table 1 indicate that with the method described in U.S. Patent No. 3,741,754 altered to feed both solid calcium and solid aluminum metal particles, calcium and aluminum recoveries both increase as the lead bath temperature increases from 500°C to 560°C. However, the results also show that there still remains a high degree of variability in test-to-test aluminum recovery; at best ± 9.6%. In addition, while the calcium recoveries are excellent, in the 90% range, this method still yields aluminum recoveries which average only 60% which are not greatly better than the other methods described in the previous prior art for adding solid aluminum metal to lead.

As mentioned previously, in preliminary experiments with the cylindrical housing, when calcium was not added, aluminum recovery was 0%. Furthermore, unreacted particles of aluminum were observed floating on the surface of the bulk lead bath outside of housing 16. This indicated that the design described in U.S. Patent No. 3,741,754 results in unreacted particles of aluminum being forced out of the open bottom of the cylindrical housing by the vortex created by the impeller. This is not a problem in the original invention described in the '180 patent when using only calcium particles since calcium dissolves quite easily and rapidly in molten lead. Aluminum, on the other hand, dissolves very slowly in molten lead and hence the aluminum reagent must be maintained in close proximity with calcium particles inside the well stirred reaction zone within the housing or bell. Particle retention time inside the housing or bell must be as long as possible to promote dissolution.

In summary, altering the method described in U.S. Patent No. 3,741,754 to allow for the addition of both solid calcium metal and solid aluminum metal into molten lead, confirmed that the localized heat released during calcium dissolution was sufficient to facilitate aluminum metal dissolution. However, the method described in this '754 patent was inappropriately designed to maximize calcium and aluminum particle retention time inside the bell or cylindrical housing. The ejection of unreacted metal particles through the open bottom of the housing was believed to be responsible for low and variable aluminum recoveries with the results being unpredictable from test-to-test.

Fig. 2 shows the preferred embodiment of apparatus in accordance with the invention which has been found to overcome the shortcomings of the prior art apparatus of Fig. 1.

In Fig. 2, two supply chutes 111 and 112 are provided from two separate hoppers 111a and 112a for calcium and aluminum particles or for calcium/aluminum alloy particles. These chutes pass into the otherwise closed top 113 of tubular housing 116 having an open bottom end outlet 117. The chutes can, if required, also be used for the introduction of a protective inert gas into the top of the housing. The housing and chutes are carried by a frame part 124 which can be moved into place as required over a vessel 125 containing the molten lead, the upper surface of which is indicated at 132.

The closed top 113 accommodates drive shaft 129 of motor 130 which carries impeller 128 at its lower end.

The housing 116 has a series of slots 118 around its periphery, which provide inlet means located at relatively small depth below the surface 132 of the lead; i.e. a depth which is small relative to that of the bottom outlet 117. A downwardly diverging frusto-conical deflector or canopy 119 is fixed to the outer surface of the housing 116 just above the slots 118; this ensures that melt entering the slots is not contaminated with surface dross or the like.

The essential differences between this invention and that of the '754 patent lie in the nature of the impeller 128 and the design of the housing 116. The impeller, instead of being a marine or axial flow type propeller, as shown in the '754 patent, is at least partially of the centrifugal flow type. Specifically, the blades of the impeller are set at an angle of between 40° and 50° to the horizontal impeller plane, preferably about 45°; rather than the shallower angle usual with axial flow type impellers. Accordingly, Applicants' impeller provides both substantial radial flow as well as axial flow; axial flow ensures that lead is moved through the housing while centrifugal flow ensures that it is swirled around in the housing long enough to become alloyed with the calcium and aluminum. An impeller of this kind may be termed a modified turbine impeller. Also, while the axial flow impeller in the '754 patent was more than two thirds the internal diameter of the housing, in the present invention the impeller diameter is less than one-half the diameter of the cylindrical portion of the housing 116 and is preferably slightly smaller than the diameter of the bottom outlet. Furthermore, while in the '754 patent the housing is wholly cylindrical in shape, applicants' housing 116 is cylindrical in the upper portion and constricted by a frusto-conical lower section 116a. This constriction impedes the flow of liquid metal out of the bottom outlet thereby further promoting radial flow inside the housing and reducing axial flow which has been shown in the preliminary experiments with the cylindrical housing 16 to result in low, unpredictable aluminum recoveries due to undissolved aluminum particles being discharged through the bottom opening.

In operation, the combined effects of a turbine type impeller 128 rotating at sufficient speed e.g. about 400-600 rpm and the constricted frusto-conical lower housing 116a cause the lead to flow in both axial and radial directions as indicated by the arrows with lead entering inlets 118, being swirled around by the impeller, and finally leaving from the bottom opening. Calcium and aluminum particles are fed simultaneously or in close sequence into the interior of the housing via chutes 111 and 112. It will be seen that the turbine impeller in combination with the frusto-conical constriction create a vortex with sufficient radial flow such that particles of the feed metals are caused to swirl around within the housing between the wall and the impeller, and above the impeller, and this ensures close proximity of the calcium and aluminum particles and maximizes their retention time within the housing. During this motion the exothermic reaction between the calcium and the lead heats the lead within the housing and adjacent to the particles and this causes dissolving of the aluminum.

During the operation, protective gas if desired can be introduced into the housing through chutes 111 and 112 or by a separate inlet port. While the use of a protective gas is not essential, tests show that use of an inert gas such as argon will improve calcium recovery by as much as 15 to 20%.

Tests, described below, have shown that results achieved with the method and apparatus as described, in terms of aluminum recovery in particular, are much better than with apparatus as shown in the '754 patent.

### EXAMPLE 1:

A conical housing similar to that shown in Fig. 2 was inserted into a 1250 kg molten lead bath. The lead melt was initially maintained at 560°C. 1.45 kg of calcium metal particles and 0.21 kg of aluminum metal particles were added simultaneously to the lead vortex generated with the impeller operating at 600 rpm inside the conical reaction housing. The reagents were introduced into the melt over a 7 to 8 minute time interval. Stirring inside the housing continued for up to 20 minutes from the start of reagent feeding. Samples were taken for chemical spectrographic analysis from the bulk lead pool outside the housing at 0, 5, 10 and 20 minute intervals from the start of reagent feeding. The results below indicate that, with the housing and impeller combination with this preferred embodiment, calcium recovery reached 92.7% by 10 minutes and 96.1% after 20 minutes. Aluminum recovery is exceptionally high reaching 81.6% at 10 minutes and increased to 82.7% after 20 minutes.

The change in calcium and aluminum levels between 10 and 20 minutes is considered insignificant; hence dissolution with the housing was complete at 10 minutes, that is within 2 to 3 minutes after end of reagent feeding.

### EXAMPLE 2:

The exact same experiment as described in Example 1 was repeated to confirm calcium and aluminum particle dissolution and recovery with the apparatus of this invention as described. Once again, dissolution was complete at the 10 minute mark, that is within 2 to 3 minutes after the end of reagent feeding. Final calcium analyzed at 1050 ppm (92.3% recovery) and the aluminum analyzed at 165 ppm (98.2% recovery).

These results confirmed that the constricted frusto-conical housing and impeller arrangement of this preferred embodiment of the invention significantly increases the recovery of aluminum encountered with the prior art arrangement. With this preferred embodiment of the present invention aluminum recoveries increased to between 83 to 98% which is substantially higher than either the 60% aluminum recoveries achieved with the cylindrical housing design in the '754 patent or the aluminum recoveries reported in the other prior art cited in this disclosure. This is attributed to the tangential fluid flow developed inside the new housing which ensures the close proximity of the aluminum and calcium particles at the periphery of the housing and increases particle retention time inside the housing. Both of these factors are necessary if the localized heat released during calcium dissolution in lead is to be effectively recovered and used to promote aluminum metal dissolution at lead melt temperatures below 660°C. No unreacted aluminum particles were observed in the bulk metal pool outside the housing when the new arrangement was used as was the case with the prior cylindrical housing of the prior patent.

A second embodiment of this invention as shown in Fig. 3, in which the same reference numerals are used for parts which are the same as those of Fig. 2. The Fig. 3 arrangement allows for the turbine impeller 228 to be located approximately at the elevation where the cylindrical portion of the housing meets the constricted portion 216a. As in the preferred embodiment, the impeller design and the frusto-conical lower section of the housing promote combined axial and radial flow patterns as shown by the arrows in Fig. 3. In this case, however, it has been found that raising the position of the impeller results in a reversal of the metal flow with liquid lead flowing in through the bottom opening and out the top openings. As before, rotating impeller 228 at sufficient speed e.g. about 400 to 600 rpm, in combination with the conical design of the housing, creates flow patterns whereby the feed metal particles swirl around within the housing between the wall and the impeller. However, in this embodiment, the buoyant forces acting on the calcium and aluminum particles may act to cause them to float out of the housing through the top openings. The design of the frusto-conical canopy 119 ensures that any undissolved particles exiting through the upper holes are caught prior to floating to the surface of the melt where they would be unrecovered due to oxidation. Nevertheless, this embodiment does not ensure as close a proximity of calcium and aluminum particles and as long a retention time within the housing as the preferred embodiment.

Tests described below with this less preferred embodiment show excellent reagent recoveries. While the recovery of aluminum is significantly better than either the preliminary experiments with the cylindrical housing as described in the '754 patent or those reported in the other prior art, it is somewhat below that reported in Example 2 with the preferred embodiment of this invention.

### EXAMPLE 3:

A conical housing similar to that shown in Fig. 3 was inserted into a 1250 kg molten lead bath. The lead melt was initially maintained at 560°C. 1.48 kg of calcium metal particles and 0.21 kg of aluminum metal particles were added simultaneously to the lead vortex generated with the impeller operating at 600 rpm inside the conical reaction housing. The reagents were introduced into the melt over a 7 to 8 minute time interval. Stirring inside the housing continued for up to 20 minutes from the start of reagent feeding. Samples were taken for chemical spectrographic analysis from the bulk lead pool outside the housing at 0, 5, 10 and 20 minute intervals from the start of reagent feeding. The results below indicate that, with the housing and impeller combination of this invention, calcium recovery reached 92.7% by 10 minutes and 96.1% after 20 minutes. Aluminum recovery reached 83.2% at 10 minutes and remained unchanged after 20 minutes.

| Sample Time | Analysis, ppm | | Recovery, % | |
|---|---|---|---|---|
| | Ca | Al | Ca | Al |
| 10 | 1100 | 140 | 92.7% | 83.2% |
| 20 | 1140 | 140 | 96.1% | 83.2% |

The 40 ppm increase in calcium levels between 10 and 20 minutes is considered insignificant; hence dissolution with the housing was complete at 10 minutes, that is within 2 to 3 minutes after end of reagent feeding.

### EXAMPLE 4:

The exact same experiment as described in Example 3 was repeated to determine the reproducibility of calcium and aluminum particle dissolution and recovery with the apparatus of this invention. Once again, dissolution was complete at the 10 minute mark, that is within 2 to 3 minutes after the end of reagent feeding. At 10 minutes, the calcium analyzed at 1068 ppm (90% recovery) and the aluminum analyzed at 140 ppm (83.2% recovery).

The results using the present invention as reported in Examples 1, 2, 3 and 4 confirm that the combination of a turbine impeller rotated at sufficient speed and a housing constricted by a frusto-conical section at its base result in substantial improvements in aluminum recovery, as compared to what can be achieved with the apparatus of the '754 patent. The position of the impeller inside the housing and the design of the impeller will determine the direction of metal flow that is either in from the top and out the bottom or vice versa. Aluminum recovery is substantially better than the prior art with both design modifications.

The improvement in recovery is attributed to the radial flow developed inside the new housing design which ensures close proximity of the aluminum and calcium particles and increases particle retention time inside the housing. Both of these factors are necessary if the localized heat released by calcium dissolution in lead is to be effectively recovered and used to promote aluminum metal dissolution at lead melt temperatures below 660°C. Aluminum recoveries were between 38% to 63% higher with the present invention compared to those obtained with experiments utilizing the cylindrical housing of the '754 patent.

Furthermore, with the present invention no unreacted aluminum particles were observed in the bulk metal pool as was the case with the cylindrical housing of the prior patent.

The results obtained with the Fig. 3 arrangement indicate that use of a turbine type impeller, i.e. one designed to cause some axial flow, is not essential, since overall flow occurs against the downwards flow direction imparted by the impeller. Accordingly, it is believed that a straight-bladed, centrifugal-type impeller, suitably positioned in the housing, could also provide satisfactory results.

## Claims

1. A process for making a lead-calcium alloy by adding calcium and aluminum materials to molten lead, and which uses a severally vertical tubular housing for mixing the material with lead, said housing having a movable support therefor and having a wall with top opening means and having a bottom opening, comprising:
placing the movable support over a vessel containing a batch of the molten lead, so that said wall of said tubular housing extends down into the molten lead sufficiently far so that the top opening means are below the surface of the lead;
feeding particles of calcium and aluminum metal or alloys thereof into the interior of said tubular housing; and
using a rotary impeller positioned in said tubular housing between its top opening means and bottom opening to cause the molten lead to be drawn from the vessel into the housing and no be returned back into the vessel, said impeller being at least partially of the centrifugal flow type and having a diameter less than one half the maximum diameter of the housing;
the shape of the housing and the nature and position of the impeller being such as to ensure that molten lead carrying the particles is swirled against the housing wall and recirculated within the housing before the lead leaves the housing.

2. A process according to claim 1, wherein the impeller, and its position in the housing, is such that the lead is drawn in through the top opening means, and, after mixing with the materials, leaves the housing through the bottom opening, and wherein flow through the bottom opening is impeded by providing a constriction in the lower part of the tubular member.

3. A process according to claim 1, wherein the temperature of the lead is less than 660°C.

4. A process according to claim 2, wherein a major part of the swirling of said particles takes place above said impeller in a downwardly converging zone of said tubular member, the impeller being positioned below the mid-point of said converging zone.

5. Apparatus for introducing calcium and aluminum into a bath of molten lead, comprising:
a generally vertical tubular housing and support means which are movable over a vessel containing a batch of molten lead for positioning the tubular housing so that an upper portion thereof is above a surface of the lead while a lower portion is submerged in the lead, said lower portion having a wall with top openings capable of being held a predetermined depth below said surface, said lower portion having a bottom opening at its lower end capable of being positioned at a depth below said surface which is larger than said predetermined depth;
supply means for feeding particles of calcium and aluminum metal or alloys thereof into the upper portion of the housing, and
an impeller mounted on a rotary shaft extending down into the housing at a position between said top and bottom openings, said impeller being at least partially of the centrifugal low type and having a diameter less than one half the maximum diameter of the housing;
wherein the shape of the housing and the nature and position of the impeller are such as to ensure that molten lead is continually drawn from the vessel into the housing and returned back into the vessel and lead carrying the particles is swirled against the housing wall and recirculated within the housing before the lead leaves the housing.

6. Apparatus according to claim 5, wherein the tubular member is constricted at a lower end portion.

7. Apparatus according to claim 5, wherein said top openings are shrouded with a canopy extending downwardly and outwardly from above said top openings.

8. Apparatus for introducing calcium and aluminum into a bath of molten lead, comprising:
a generally vertical tubular housing and support means which are movable over a vessel containing a batch of molten lead for positioning the tubular housing so that an upper portion thereof is above a surface of the lead while a lower portion is submerged in the lead, said lower portion having a wall with top openings capable of being held a predetermined depth below said surface, said lower portion having a bottom opening at its lower end capable of being positioned at a depth below said surface which is larger than said predetermined depth;
supply means for feeding particles of calcium, and aluminum metal or alloys thereof into the upper portion of the tubular housing, and
an impeller mounted on a rotary shaft extending down into the tubular housing at a position between said top and bottom openings, said impeller being at least partially of the centrifugal flow type and having a diameter less than one half the maximum diameter of the housing, and being capable of drawing molten lead into the housing through said top openings and returning it to the vessel through the bottom openings;
wherein the lower portion of the tubular housing converges downwardly to said bottom opening, and wherein the impeller is positioned at or within the downwardly converging lower portion of the housing.

9. Apparatus according to claim 8, wherein said top openings are shrouded with a canopy extending downwardly and outwardly from above said top openings.

10. Apparatus according to claim 8, wherein said impeller has blades set at between 40° and 50° to the impeller plane.

11. Apparatus according to claim 8, wherein said impeller diameter is less than the internal diameter of the bottom opening of the housing.

12. Apparatus according to claim 8, wherein the impeller is situated closer to the bottom outlet than to a mid-point of zinc downwardly converging portion.

13. Apparatus according to claim 8, wherein the bottom opening is between one half and one third the diameter of the upper portion of the housing.

## Patentansprüche

1. Verfahren zur Herstellung einer Blei-Kalzium Legierung durch Zugabe von Kalzium und Aluminium Material zu geschmolzendem Blei, unter Verwendung eines im wesentlichen vertikalen, röhrenförmigen Gehäuses zur Mischung des Materials mit Blei, wozu das Gehäuse einen beweglichen Träger aufweist,
sowie eine Wandung mit oberen Öffnungseinrichtungen und mit einer Bodenöffnung, mit folgenden Schritten:
- der bewegliche Träger wird derart über einem Behälter mit einer Menge des geschmolzenen Bleis positioniert, daß die Wandung des röhrenförmigen Gehäuses sich nach unten ausreichend weit in das geschmolzene Blei erstreckt, so daß die oberen Öffnungseinrichtungen unterhalb der Oberfläche des Bleis zu liegen kommen;
- Partikel des Kalziums und des Aluminiummetalls oder deren Legierungen werden in das Innere des röhrenförmigen Gehäuses eingebracht;
- ein rotierendes Flügelrad, das im röhrenförmigen Gehäuse zwischen dessen oberen Öffnungseinrichtungen und dessen Bodenöffnung gehalten ist, wird dazu verwendet, um das geschmolzene Blei aus dem Behälter in das Gehäuse zu fördern und wieder dorthin zurückzubringen, wobei dieses Flügelrad zumindest teilweise vom Radialtyp ist und einen Durchmesser aufweist, der weniger als die Hälfte des maximalen Durchmessers des Gehäuses beträgt;
- die Form des Gehäuses und die Bauart und Positionierung des Flügelrades werden so gewählt, daß sichergestellt ist, daß geschmolzenes Blei, das die Partikel mitnimmt, gegen die Wandung des Gehäuses geschleudert und innerhalb des Gehäuses zurückgeführt wird, bevor das Blei das Gehäuse verläßt.

2. Verfahren nach Anspruch 1, wobei das Flügelrad und seine Positionierung im Gehäuse derart gewählt ist, daß das Blei durch die oberen Öffnungseinrichtungen hereingezogen wird und nach der Mischung mit den Materialien das Gehäuse über die Bodenöffnung verläßt, und wobei der Durchfluß durch die Bodenöffnung durch eine Verengung im unteren Teil des röhrenförmigen Bauteils beschleunigt wird.

3. Verfahren nach Anspruch 1, wobei die Temperatur des Bleis unterhalb von 660°C liegt.

4. Verfahren nach Anspruch 2, wobei der größere Teil der Verwirbelung der genannten Partikel oberhalb des Flügelrades in einem sich nach unten verengenden Bereich des röhrenförmigen Bauteils stattfindet, und wobei das Flügelrad unterhalb der Mitte des sich verengenden Bereichs positioniert ist.

5. Vorrichtung zur Einbringung von Kalzium und Aluminium in ein Bad aus geschmolzendem Blei, mit folgenden Bestandteilen:
- ein im wesentlichen vertikales röhrenförmiges Gehäuse und Trägervorrichtungen, die über einen Behälter mit einer Ladung geschmolzenem Blei bewegbar sind, um das röhrenförmige Gehäuse derart zu positionieren, daß ein oberer Abschnitt desselben oberhalb einer Oberfläche des Bleis zu liegen kommt, wogegen ein unterer Abschnitt in das Blei eingetaucht wird, mit einer Wandung mit oberen Öffnungen des unteren Abschnitts, die in einer vorgebbaren Tiefe unterhalb dieser Oberfläche gehalten werden können, wobei der untere Abschnitt eine Bodenöffnung an seinem unteren Ende aufweist, die bei der Tiefe unterhalb dieser Oberfläche positionierbar ist, die größer ist als die vorgegebene Tiefe;
- Zuführeinrichtungen zur Einbringung von Partikeln von Kalzium oder Aluminiummetall oder Legierungen davon in den oberen Abschnitt des Gehäuses, und
- ein Flügelrad, das auf einer rotierenden Welle sitzt und sich in das Gehäuse hinein bis zu einer Position zwischen den oberen und unteren Öffnungen erstreckt, wobei das Flügelrad zumindest teilweise vom Radialtyp ist und einen Durchmesser aufweist, der weniger als die Hälfte des Maximaldurchmessers des Gehäuses aufweist, wobei die Form des Gehäuses und die Bauart und Positionierung des Flügel rads so gewählt werden, daß sichergestellt ist, daß geschmolzenes Blei kontinuierlich aus dem Behälter in das Gehäuse gefördert und zurückgeführt wird, und daß Blei, das die Partikel trägt, gegen die Wandung des Gehäuses geschleudert und innerhalb des Gehäuses zurückgeführt wird, bevor das Blei das Gehäuse verläßt.

6. Vorrichtung nach Anspruch 5, wobei das röhrenförmige Bauteil an seinem unteren Abschnitt verjüngt ist.

7. Vorrichtung nach Anspruch 5, wobei die oberen Öffnungen mit einer Haube abgedeckt sind, die sich nach unten und nach außen von den oberen Öffnungen erstreckt.

8. Vorrichtung zur Einbringung von Kalzium und Aluminium in ein Bad aus geschmolzenem Blei, mit folgenden Bestandteilen:
- ein im wesentlichen vertikales röhrenförmiges Gehäuse und Trägervorrichtungen, die über einen Behälter mit einer Ladung geschmolzenem Blei bewegbar sind, um das röhrenförmige Gehäuse derart zu positionieren, daß ein oberer Abschnitt desselben oberhalb einer Oberfläche des Bleis zu liegen kommt, wogegen ein unterer Abschnitt in das Blei eingetaucht wird, mit einer Wandung mit oberen Öffnungen des unteren Abschnitts, die in einer vorgebbaren Tiefe unterhalb dieser Oberfläche gehalten werden können, wobei der untere Abschnitt eine Bodenöffnung an seinem unteren Ende aufweist, die bei der Tiefe unterhalb dieser Oberfläche positionierbar ist, die größer ist als die vorgegebene Tiefe;
- Zuführeinrichtungen zur Einbringung von Partikeln von Kalzium oder Aluminiummetall oder Legierungen davon in den oberen Abschnitt des Gehäuses, und
- ein Flügelrad, das auf einer rotierenden Welle sitzt und sich in das Gehäuse hinein bis zu einer Position zwischen den oberen und unteren Öffnungen erstreckt, wobei das Flügelrad zumindest teilweise vom Radialtyp ist und einen Durchmesser aufweist, der weniger als die Hälfte des Maximaldurchmessers des Gehäuses aufweist,und der in der Lage ist, geschmolzenes Blei über die oberen Öffnungen in das Gehäuse zu fördern und es über die Bodenöffnungen wieder in den Behälter zurückzuführen, wobei der untere Abschnitt des röhrenförmigen Gehäuses sich nach unten zur Bodenöffnung hin verjüngt, und
wobei das Flügelrad an oder innerhalb des sich verjüngenden unteren Abschnitts gehalten ist.

9. Vorrichtung nach Anspruch 8, wobei die oberen Öffnungen mit einer Haube abgedeckt sind, die sich nach unten und nach außen von den oberen Öffnungen erstreckt.

10. Vorrichtung nach Anspruch 8, wobei das Flügelrad Blätter aufweist, die gegenüber der Flügelradebene zwischen 40° und 50° geneigt angeordnet ist.

11. Vorrichtung nach Anspruch 8, wobei der Durchmesser des Flügelrades weniger als der Innendurchmesser der Bodenöffnung des Gehäuses beträgt.

12. Vorrichtung nach Anspruch 8, wobei das Flügelrad näher zum bodenseitigen Auslaß als zur Mitte des sich nach unten verjüngenden Abschnitts angeordnet ist.

13. Vorrichtung nach Anspruch 8, wobei die Bodenöffnung zwischen einer Hälfte und einem Drittel des Durchmessers des oberen Abschnitts des Gehäuses ausmacht.

## Revendications

1. Procédé pour fabriquer un alliage plomb-calcium en ajoutant à du plomb fondu des matériaux de calcium et d'aluminium et qui emploie un logement tubulaire généralement vertical pour mélanger le matériau avec le plomb, ledit logement étant muni d'un support mobile et ayant une paroi dotée de moyens d'ouverture hauts et ayant une ouverture basse, comprenant les étapes consistant à:
placer le support mobile au-dessus d'un récipient contenant un bain du plomb fondu, de manière que ladite paroi dudit logement tubulaire descende dans le plomb fondu suffisamment loin pour que le moyen d'ouverture du haut soit au-dessous de la surface du plomb;
charger les particules de calcium et d'aluminium métal ou d'alliages d'aluminium dans l'intérieur dudit logement tubulaire; et
employer une hélice rotative placée dans ledit logement tubulaire entre ses moyens d'ouverture hauts et son ouverture basse pour aspirer le plomb fondu du récipient dans le logement et le renvoyer dans le récipient, ladite hélice étant au moins partiellement du type à écoulement centrifuge et ayant un diamètre inférieur à la moitié du diamètre maximum du logement;
la forme du logement et la nature et la position de l'hélice étant susceptibles de garantir que le plomb fondu portant les particules est conformé en un tourbillon contre la paroi du logement et est recirculé au sein du logement avant que le plomb quitte le logement.

2. Procédé selon la revendication 1, dans lequel l'hélice, et sa position dans le logement, sont telles que le plomb est aspiré dans le logement à travers les moyens d'ouverture hauts et, après mélange avec les matériaux, quitte le logement à travers l'ouverture basse, et dans lequel l'écoulement à travers l'ouverture basse est gêné grâce à un étranglement dans la partie inférieure de l'élément tubulaire.

3. Procédé selon la revendication 1, dans lequel la température du plomb est inférieure à 660°C.

4. Procédé selon la revendication 2, dans lequel une majeure partie du tourbillon desdites particules se fait au-dessus de ladite hélice dans une zone convergeant de haut en bas dudit élément tubulaire, l'hélice étant placée au-dessous du point médian de ladite zone convergente

5. Appareil pour introduire du calcium et de l'aluminium dans un bain de plomb fondu, comprenant:
un logement tubulaire généralement vertical et un moyen de support qui sont mobiles au-dessus d'un récipient contenant un bain de plomb fondu pour positionner le logement tubulaire de manière que sa partie supérieure soit au-dessus de la surface du plomb tandis que sa partie inférieure est immergée dans le plomb, ladite partie inférieure possédant une paroi munie d'ouvertures hautes capables d'être maintenues à une profondeur prédéterminée au-dessous de ladite surface, ladite partie inférieure étant munie d'une ouverture basse, à son extrémité inférieure, capable d'être positionnée à une profondeur, au-dessous de ladite surface, qui soit plus grande que ladite profondeur prédéterminée;
un moyen d'alimentation pour charger les particules de calcium et d'aluminium métal ou d'alliages d'aluminium dans la partie supérieure du logement; et
une hélice montée sur un axe rotatif qui descend dans le logement à une position entre lesdites ouvertures hautes et basse, ladite hélice étant au moins partiellement du type à écoulement centrifuge et ayant un diamètre inférieur à la moitié du diamètre maximum du logement;
dans lequel la forme du logement et la nature et la position de l'hélice sont susceptibles de garantir que le plomb fondu est aspiré en continu du récipient dans le logement et renvoyé dans le récipient et que le plomb portant les particules est conformé en un tourbillon contre la paroi du logement et est recirculé au sein du logement avant que le plomb quitte le logement.

6. Appareil selon la revendication 5, dans lequel l'élément tubulaire est étranglé au niveau de sa partie inférieure.

7. Appareil selon la revendication 5, dans lequel lesdites ouvertures hautes sont coiffées par un auvent s'étendant de haut en bas et vers l'extérieur depuis le dessus desdites ouvertures hautes.

8. Appareil pour introduire du calcium et de l'aluminium dans un bain de plomb fondu, comprenant:
un logement tubulaire généralement vertical et un moyen de support qui sont mobiles au-dessus d'un récipient contenant un bain de plomb fondu pour positionner le logement tubulaire de manière que sa partie supérieure soit au-dessus de la surface du plomb tandis que sa partie inférieure est immergée dans le plomb, ladite partie inférieure possédant une paroi munie d'ouvertures hautes capables d'être maintenues à une profondeur prédéterminée au-dessous de ladite surface, ladite partie inférieure étant munie d'une ouverture basse, à son extrémité inférieure, capable d'être positionnée à une profondeur, au-dessous de ladite surface, qui soit plus grande que ladite profondeur prédéterminée;
un moyen d'alimentation pour charger les particules de calcium et d'aluminium métal ou d'alliages d'aluminium dans la partie supérieure du logement; et
une hélice montée sur un axe rotatif qui descend dans le logement tubulaire à une position entre lesdites ouvertures hautes et bases, ladite hélice étant au moins partiellement du type à écoulement centrifuge et ayant un diamètre inférieur à la moitié du diamètre maximum du logement, et étant capable d'aspirer le plomb fondu dans le logement à travers lesdites ouvertures hautes et de le renvoyer dans le récipient à travers les ouvertures basses;
dans lequel la partie inférieure du logement tubulaire converge de haut en bas vers ladite ouverture basse et dans lequel l'hélice est placée au niveau de la partie inférieure, convergente de haut en bas, du logement ou à l'intérieur de cette partie inférieure.

9. Appareil selon la revendication 8, dans lequel lesdites ouvertures hautes sont coiffées par un auvent s'étendant de haut en bas et vers l'extérieur depuis le dessus desdites ouvertures hautes.

10. Appareil selon la revendication 8, dans lequel ladite hélice possède des lames réglées à entre 40° et 50° par rapport au plan de l'hélice.

11. Appareil selon la revendication 8, dans lequel ledit diamètre de l'hélice est inférieur au diamètre intérieur de l'ouverture basse du logement.

12. Appareil selon la revendication 8, dans lequel l'hélice est située plus près de la sortie basse que du point médian de la partie convergente de haut en bas.

13. Appareil selon la revendication 8, dans lequel l'ouverture basse est entre la moitié et le tiers du diamètre de la partie supérieure du logement.
